

## UNITED STATES PATENT OFFICE

2,104,641

## LUBRICATING PREPARATION

Hugh Francis Green, York, England

No Drawing. Application August 5, 1935, Serial  
No. 34,842. In Great Britain December 5,  
1934

8 Claims. (Cl. 87—9)

This invention relates to improved lubricating preparations containing oils.

It is one object of the invention to provide an improved penetrating oil for creeping in between the leaves of leaf springs, easing rusted screw-threads and like purposes, and in particular to provide a composition more nearly of the consistency of gear oil than of an ordinary penetrating oil and yet having the property of creeping between the leaves of springs and thereafter remaining between them and performing the functions of an efficient lubricant.

It is believed however, that the composition hereinafter to be described will find many other applications and with obvious modifications, such as the selection of different types of lubricating oils, it is believed that the composition according to the invention will be suitable for a variety of purposes. Thus the invention may result in a lowering of the temperature at which oil solidifies, hence enabling the oil to be used in climates or for purposes, such as refrigeration, which involve lubrication at low temperatures, and in this latter connection for such purposes as power transmission liquids.

A lubricating preparation according to the present invention comprises a lubricating oil and a neutralized hydroxy acid.

The neutralized hydroxy acid may be a salt or an ester or in certain cases, a mixture of a salt and an ester of the same or different hydroxy acids. Where a salt is employed the ester of another hydroxy acid may be employed as a solubilizing agent in order to bring about compatibility between the oil and the hydroxy acid salt. Esters other than hydroxy acid esters, however, may be employed with a hydroxy acid salt to render the latter compatible with the oil, for example, amyl acetate and the glycerol esters of higher fatty acids such as palmitic, oleic or stearic acids.

According to one feature of the invention, the neutralized hydroxy acid is an alkali salt of a hydroxy derivative of cholanic acid,  $C_{24}H_{40}O_2$ . Examples of such acids are glyco cholic acid



and tauro cholic acid



These two acids are constituents of the bile fluid and are known as bile acids. A pharmaceutical preparation from the bile of oxen which contains both these acids is known as sodium tauro glyco cholate.

According to another feature of the invention, a lubricant comprises a lubricating oil and a hydroxy acid ester such as a lactic acid ester. Where a lactic ester is employed, according to a preferred feature of the invention, it serves as a solvent for a hydroxy derivative of cholanic acid such as sodium or potassium tauro glyco cholate. In this case, the lactic acid ester employed is preferably that of an aliphatic alcohol higher than that of butyl alcohol, i. e. an aliphatic alcohol containing more than 4 carbon atoms, since it is found that if butyl or ethyl lactate are employed the mixture may slowly separate into a clear upper zone and a cloudy lower zone. Amyl lactate has been found to be satisfactory and produces a slightly cloudy oil in which no separation appears to occur. Higher lactates, whether of primary, secondary or tertiary alcohols may also be employed. The lactic acid ester is, of course, preferably employed in proportions just sufficient to bring about compatibility between the lubricating oil and the bile salts.

The invention also includes the process for producing the improved lubricant which consists in adding a solution, in a solubilizing agent, of a soluble salt to a lubricating oil, for example, the addition of a solution of sodium tauro glyco cholate in amyl lactate to a mineral lubricating oil.

The invention further includes the incorporation with the composition hereinbefore described of graphite preferably in colloidal condition.

In carrying out the invention, the hydroxy acid salt or ester, or both, may be added to a thick lubricating oil or it may be added as a constituent in a known penetrating oil comprising a comparatively heavy mineral oil to which kerosene and amyl acetate are added. In such known penetrating oils as hitherto prepared in order to obtain the desired fluidity and sufficient penetrating power, the proportions of kerosene and amyl acetate added have been substantial, and it has been necessary to add graphite to the mixture to obtain sufficient lubricating properties. In preparing such liquid in accordance with the present invention, the penetrating power of a thick lubricating oil can be so increased by a very small proportion of the hydroxy acid that the amount of kerosene and graphite may be either substantially reduced or dispensed with altogether.

The following examples illustrate the nature of the invention though it will be appreciated that the proportions given may be varied in each case:—

*Example 1*

5 A concentrated solution of sodium tauro glyco cholate in amyl lactate was employed at room temperature. This was mixed with an oil consisting of three parts of mineral oil, sold under the name Colza mineral vaclite, and five parts of oil sold under the trade name Etmar medium heavy. Two drams of the concentrated solution of bile salts was added to each pint of the mixed 10 oils. This produced a penetrating oil suitable for the lubrication of leaf springs, softening and loosening rust and like purposes.

*Example 2*

15 15 Two drams of the same solution of bile salts as in Example 1 was added to one pint of thick gear oil sold under the name Mobiloil C. This results in a black thick oil which can be used for lubrication of leaf springs by painting it on 20 the sides thereof when it will slowly creep in between the leaves and remain there for a considerable period.

*Example 3*

25 25 This is an example of the application of the invention to the preparation of a penetrating oil containing kerosene and amyl acetate. The proportions of the constituents were as follows:—

30 Lubricating oil sold as Rimer's heavy grade  
H oil \_\_\_\_\_ounces 5½  
Kerosene \_\_\_\_\_do 4½  
Amyl acetate \_\_\_\_\_dram ½  
Concentrated solution of sodium tauro glyco cholate in alcohol \_\_\_\_\_dram 1  
35 Graphite in the form sold as Rimer's graphite suspension (running-in compound) \_\_\_\_\_dram 1

Instead of the alcohol neutral esters such as 40 the glycerol esters of palmitic, oleic or stearic acids may be used as solvent for the tauro glyco cholate.

What I claim as my invention and desire to secure by Letters Patent is:—

1. A lubricating preparation comprising a lubricating oil, a salt of a bile acid and a liquid lactate of an aliphatic alcohol having more than 5 four carbon atoms.

2. A lubricating preparation comprising a lubricating oil and sodium tauro glyco cholate and a liquid lactate of an aliphatic alcohol having more than four carbon atoms, in sufficient quantity 10 to form a compatible solution with the lubricating oil.

3. A lubricating preparation consisting of a lubricating oil and more than 0.1% of sodium tauro glyco cholate dissolved in sufficient amyl 15 lactate to form a compatible solution with the lubricating oil.

4. A lubricating preparation comprising a lubricating oil and sodium tauro glyco cholate and sufficient amyl lactate to form a compatible solution 20 with the lubricating oil.

5. A lubricating preparation comprising a mineral lubricating oil and sodium tauro glyco cholate and sufficient amyl lactate to form a compatible solution with the mineral lubricating oil. 25

6. A process for preparing a lubricating preparation which comprises dissolving a salt of a bile acid in amyl lactate and adding the said solution to a lubricating oil.

7. A process for preparing a lubricating preparation which comprises dissolving a salt of a bile acid in amyl lactate and adding the said solution to a mineral lubricating oil. 30

8. A process for preparing a lubricating preparation which comprises dissolving sodium tauro glyco cholate in sufficient amyl lactate to form a compatible solution with a mineral lubricating oil and adding the said solution to the lubricating oil. 35

HUGH FRANCIS GREEN. 40